

# United States Patent Office

2,796,369

Patented June 18, 1957

1

2,796,369

## METHOD OF PROTECTING ZINC-COPPER ALLOYS AGAINST CORROSION AND PRODUCT THEREOF

Allan E. Chester, Highland Park, and Bruno R. Jeremias, Chicago, Ill., and Joseph T. Irwin, Lakewood, Ohio, assignors to Poor & Company, Chicago, Ill., a corporation of Delaware

No Drawing. Application April 15, 1953,  
Serial No. 349,105

6 Claims. (Cl. 148—6.2)

This invention relates to corrosion protected articles and to a method of protecting zinc-copper alloys, more particularly white alloys of zinc and copper against corrosion.

White alloys of zinc and copper have a tendency to turn white or grayish white with age, a property sometimes referred to as "white corrosion," which is apparently due to the formation of oxides and carbonates of zinc.

Zinc surfaced articles have been protected against "white corrosion" by treating them with various types of chromic acid solutions usually followed by a secondary treatment with an alkali to remove some of the by-products formed by the primary treatment. In our copending application Serial No. 349,068, filed of even date here-with, we have described a method of protecting chromium plated zinc-copper alloy surfaced articles by treatment with an acidified aqueous solution of chromic acid. In order to obtain the desired corrosion protection it is necessary to add enough acid to produce a relatively low pH and most of these acidified chromic acid solutions when applied to the zinc-copper alloy coating which has not been over-plated with chromium cause discoloration of the surface which is especially undesirable when a bright finish of high specular reflectivity is required.

One of the objects of the present invention is to provide a method for protecting against corrosion alloys of zinc and copper regardless of whether such alloys have been over-plated with chromium.

A further object of the invention is to provide new and improved articles containing a surface coating of an alloy of zinc and copper sealed with a sealing composition which affords good protection against corrosion and does not discolor the zinc-copper alloy surface.

Another object of the invention is to provide new and improved corrosion inhibiting compositions for protecting against corrosion alloys of zinc and copper. Other objects will appear hereinafter.

In accordance with the invention it has been found that zinc-copper surfaced articles can be protected against corrosion by treating them with a solution of chromic acid ( $\text{CrO}_3$ ) and nitric acid, preferably containing an acid stable wetting agent.

The chromic acid-nitric acid solution is preferably prepared in the form of a concentrate and then diluted with water before being applied to the zinc-copper alloy surface of the article. The pH of the composition which is applied to the zinc-copper alloy surfaced article is preferably within the range of 0.75 to 1.75.

The corrosion protection treatment may be applied by spraying, dipping or in any other suitable manner, but it is preferable to immerse the article to be treated containing a zinc-copper alloy surface in a solution of the chromic acid and nitric acid composition for a short period of time. Good results can usually be obtained by immersing the zinc-copper surfaced article in such a solution for a period of 1 minute but the time period can be varied depending upon the concentration of the solution

2

and the results desired. Ordinarily at least a 10 second immersion is required in order to obtain a substantial corrosion inhibiting effect and a period of not more than 2 minutes is necessary. The treatment can be carried out at ordinary temperatures ( $20^\circ$  to  $25^\circ$  C.).

The invention will be further illustrated but is not limited by the following example.

## EXAMPLE

10 A concentrate is prepared by mixing together the following ingredients in water:

|                                                              | Ounces per gallon |
|--------------------------------------------------------------|-------------------|
| $\text{CrO}_3$                                               | 30                |
| $\text{Na}_2\text{Cr}_2\text{O}_7 \cdot 2\text{H}_2\text{O}$ | 15                |
| 68% $\text{HNO}_3$                                           | 21.5              |
| 40% aqueous solution of octyl alcohol sodium sulfate         | .85               |

This concentrate is diluted with water to produce a sealing composition containing 2% to 6% by volume of the foregoing concentrate (2-6 cc. of concentrate per 100 cc. of aqueous solution) and articles having a white zinc-copper alloy surface or a white zinc-copper alloy surface over-plated with chromium are protected against corrosion by immersing them in this composition. The optimum results are obtained with a 4% by volume solution of the concentrate at a temperature of  $20^\circ$  to  $25^\circ$  C. for an immersion period of about 1 minute.

In this composition a 2% solution by volume of the concentrate has a pH of about 1.3 and a 4% by volume solution of the concentrate has a pH of about 1.0.

In the foregoing example the octyl alcohol sodium sulfate is a wetting agent and can be omitted from the composition. Its primary purpose is to reduce the surface tension between the active effective ingredients of the composition and the zinc-copper alloy surface article. The sodium dichromate in the composition is another source of chromic acid which is formed by the reaction between the dichromate and nitric acid producing sodium nitrate as an ingredient in the composition.

The acid content should be held within relatively narrow limits as defined by the pH in order to obtain the desired results. Especially satisfactory results are obtained in the practice of the invention with white zinc-copper alloy surfaced articles having a copper content in the alloy of 10% to 20%, the remainder being zinc.

The copper content can be as low as 5% and is usually not higher than 30% by weight of the alloy. The corrosion inhibiting composition described in the foregoing example is primarily applicable to the treatment of predominantly zinc alloys of zinc and copper which have a silvery or whitish appearance and can also be applied to surfaces of such alloys that have been over-plated with chromium.

55 After the corrosion inhibiting treatment has been applied the resultant zinc-copper alloy surfaced article is rinsed simply by washing with water. No secondary treatment is required either by leaching with an alkali or otherwise.

If a wetting and penetrating agent is used in the sealing composition it should be one which is stable under the highly acid conditions and at the same time not precipitated from the bath or destroyed by the high concentration of chromic acid present in the sealing composition. Examples of suitable wetting and penetrating agents are octyl alcohol sodium sulfate, isopropyl naphthalene sodium sulfonate, the diethyl ester of sodium sulfosuccinic acid, isobutyl naphthalene sodium sulfonate, other alkylated aryl sulfonic acids, soya bean amine oxyalkylated with approximately 10 mols of ethylene oxide, containing an average of 20 carbon atoms in its alkyl chain and having an average molecular weight of 714,

and other oxyalkylated amines of long chain acids containing 8 to 60 carbon atoms in which the oxyalkyl groups are derived from ethylene oxide, 1,2-propylene oxide or mixtures thereof. The preferred wetting agents of this last mentioned type contain at least 4 mols of alkylene oxide per mol of primary fatty amine, preferably around 10 to 20 mols of alkylene oxide per mol of primary fatty amine, and are soluble and stable in acids in the concentrations employed in the practice of the invention.

The sealing composition employed in the practice of the invention preferably contains around 1 gram to 10 grams of chromium (Cr) as chromic acid ( $\text{CrO}_3$ ) per liter of solution. Smaller amounts produce a less pronounced effect and larger amounts do not substantially add to the improvement in the corrosion protection obtained and may produce discoloration.

The invention provides new and improved corrosion protected articles and makes it possible to seal a coating of a zinc and copper alloy to enhance the corrosion resistance. It is especially valuable in providing a method for enhancing the corrosion resistance of white zinc-copper alloy surfaced articles which have a high specular reflectivity because the treatment does not discolor the surface. The same is true where such articles have been over-plated with chromium and especially where the coating of chromium is non-uniform, as is often the case with contoured articles because of the poor throwing power of chromium electroplating baths. An important advantage of the treatment herein described is that it is unnecessary to heat either the zinc-copper alloy surfaced article or the sealing composition which is applied thereto. Zinc-copper alloy surfaced articles which have been treated in accordance with the practice of the invention are highly resistant to white corrosion and, in the case of ferrous metal articles, to the formation of red rust corrosion over a long period of time.

The expression "zinc-copper alloy surfaced article" is employed herein to cover any article having an exterior surface of an alloy of zinc and copper regardless of whether the article itself is made of zinc, a zinc-copper alloy, a ferrous metal, or some other metal capable of being coated with a zinc-copper alloy. The expression "zinc-copper alloy plated article" is employed herein to describe a zinc-copper alloy coated article in which the zinc-copper alloy coating has been applied by an electroplating process. The expression "white alloy of zinc and copper" is employed herein to describe alloys of zinc and copper which have a white or silvery appearance as distinguished from alloys of zinc and copper which are yellow in appearance. The expression "over-plated with chromium" is employed herein to describe an article in which a chromium layer or coating has been applied by electrodeposition over the zinc-copper alloy surfaced article.

The invention is hereby claimed as follows:

1. A process of improving corrosion resistance which comprises treating a zinc-copper alloy surfaced article

wherein the alloy contains 5% to 30% by weight copper, the remainder being zinc, with an aqueous solution consisting essentially of chromic acid and nitric acid having a pH within the range of 0.75 to 1.75 and containing 1 to 10 grams of chromium per liter of solution.

2. A process of improving corrosion resistance which comprises treating a zinc-copper alloy surfaced article wherein the alloy contains 5% to 30% by weight copper, the remainder being zinc, with an aqueous solution consisting essentially of chromic acid, sodium dichromate and nitric acid having a pH within the range of 0.75 to 1.75 and containing 1 to 10 grams of chromium per liter of solution.

3. A process of improving corrosion resistance which comprises treating a zinc-copper alloy surfaced article wherein the alloy contains 5% to 30% by weight copper, the remainder being zinc, with an aqueous solution consisting essentially of chromic acid and nitric acid, containing 1 to 10 grams of chromium per liter of solution, having a pH within the range of 0.75 to 1.75 and containing a wetting agent which is stable in said acid solution.

4. A process of improving corrosion resistance which comprises treating a zinc-copper alloy surfaced article wherein the alloy contains 5% to 30% by weight copper, the remainder being zinc, with an aqueous solution consisting essentially of chromic acid and nitric acid, containing 1 to 10 grams of chromium per liter of solution, having a pH within the range of 0.75 to 1.75 for a period of 10 seconds to 2 minutes and rinsing the resultant product with water.

5. A zinc-copper alloy surfaced article wherein the alloy contains 5% to 30% by weight copper, the remainder being zinc, inhibited against corrosion with a coating of an aqueous solution consisting essentially of chromic acid and nitric acid having a pH within the range of 0.75 to 1.75 and containing 1 to 10 grams of chromium per liter of solution.

6. A white zinc-copper alloy surfaced article wherein the alloy contains 10% to 20% by weight copper, the remainder being zinc, inhibited against corrosion with a sealing coating consisting essentially of an aqueous solution of chromic acid and nitric acid having a pH within the range of 0.75 to 1.75 and containing 1 to 10 grams of chromium per liter of solution.

#### References Cited in the file of this patent

##### UNITED STATES PATENTS

|           |                       |               |
|-----------|-----------------------|---------------|
| 2,106,904 | Wilhelm -----         | Feb. 1, 1938  |
| 2,269,435 | Buzzard -----         | Jan. 13, 1942 |
| 2,315,564 | Thompson et al. ----- | Apr. 6, 1943  |
| 2,387,494 | Bushrod -----         | Oct. 23, 1945 |
| 2,610,133 | Thomson -----         | Sept. 9, 1952 |

##### FOREIGN PATENTS

|         |                     |               |
|---------|---------------------|---------------|
| 287,450 | Great Britain ----- | Oct. 18, 1928 |
| 706,347 | Germany -----       | May 24, 1941  |